

Jan. 29, 1963

F. J. STANCAZAK ET AL

3,075,260

STEREOTYPE MAT

Filed May 9, 1955

2 Sheets-Sheet 1



Inventors  
Frank J. Stanczak  
Richard A. Wolterding  
By James Walter Anderson, Attorneys

Jan. 29, 1963

F. J. STANCAK ET AL

3,075,260

STEREOTYPE MAT

Filed May 9, 1955

2 Sheets-Sheet 2

*Fig. 4.*



*Fig. 6.*



*Fig. 5.*

Inventors  
Frank J. Stanczak  
Richard A. Wolterding  
By: Evans, Shuster & Anderson  
Attorneys

## 1

3,075,260

## STEREOTYPE MAT

Frank J. Stanczak, Easton, Pa., and Richard A. Woltering, Neenah, Wis., assignors, by mesne assignments, to Kimberly-Clark Corporation, a corporation of Delaware

Filed May 9, 1955, Ser. No. 507,113

10 Claims. (Cl. 22—5.5)

The present invention relates generally to stereotype mats and is particularly concerned with an improved composite stereotype mat and backing and with certain methods for manufacturing such products. This application is a continuation-in-part of our copending application Serial No. 349,352, filed April 17, 1953, now Patent 2,936,797, issued May 17, 1960.

In the usual process for making a stereotype mat, a paperboard mat or flong, as it is sometimes called, is laid over a lockup containing the type, engravings, and other printing elements which are to be reproduced in the stereotype plate. The lockup with the mat in position is then subjected to heavy pressure, sufficient to press the mat into the face of the lockup and provide a reproduction of the printing elements in the face of the mat. During the pressing operation, a molding combination of cork, felt, or other suitable materials is positioned intermediate the mat and the pressure element.

Following the pressing operation, the mat may be dried by a process which includes placing the imprinted mat in a curved former and dryer, sometimes termed the "scorcher." This forming and drying operation achieves several desirable results. Since the actual printing plate is made by casting molten type metal against the curved mat as a matrix, it is necessary that the mat be completely dried prior to the casting operation and that it be sufficiently hard and rigid to resist the casting pressure. In addition, it is the current practice in various printing industries to shrink stereotype mats quite substantial amounts in order to reduce the size of the printed image and the amount of paper required in the printing operation. These two functions, i.e., the preparation of the mat for the casting operation and the controlled shrinkage of that mat are accomplished during the drying operation.

The usual dryer for forming the mat receives the mat against a curved, foraminous surface, which is connected to a source of reduced pressure in order that the moisture and other vapors liberated during the heating operation will be drawn off through the back of the mat. When using a high shrink mat, it is normally desirable for the drying to be done in two steps, in the first of which the mat is heated while still flat to drive off some of the moisture and, in the second step, the mat is formed into a curved shape in the dryer mentioned above and is heated under vacuum conditions to drive off the remaining moisture through the back of the mat. In this way, the maximum shrinkage of the mat is achieved. In a low-shrink or a non-shrink mat the pre-drying step prior to placing the mat in the former is generally not required.

Since the forming and casting operations involve quite substantial pressures, it has been found necessary to provide some means for preventing buckling or yielding of the mat in the nonprinting areas, and particularly those areas which are of substantial dimensions. In practice, the most common means for packing or backing the mat consists in attaching thin strips of paper felt along the rear surface of the mat in those areas of the mat which have rather large nonprinting areas. This hand packing is usually done after the mat has been molded and, if a pre-drying step is used, between the first drying and the final drying against the curved former. Reinforcement of nonprinting areas too small to be packed with felt

## 2

strips is sometimes accomplished by running the point of a pencil on the back side of the mat in those areas to form nonplanar areas in the face of the mat which will resist buckling more effectively.

5 Packing operations of the type mentioned above constitute a very serious problem in the newspaper field. Mat packing is inherently time consuming and costly and, of even greater importance, it must be done shortly before press time, when every minute is vital. Many of the 10 pages of the newspaper cannot be completed in the lock-up until a few minutes before press time, either because it is desired to cover last minute developments or because of the time necessary to complete the stereoplates that make up portions of the pages. Consequently, when such 15 pages are finally closed, and there may be many such pages in a large newspaper, it is necessary that the stereotype mat be promptly finished so that the plates for the presses can be cast and installed. At this point, the necessity heretofore for hand packing each of the mats has been a serious deterrent to prompt completion of such 20 mats. The hand packing operation is time consuming and requires the services of skilled workmen who must use considerable judgment in selecting the areas to be packed and in applying the packing material properly, in 25 order to render the packing effective for its intended purpose. Consequently, this type of packing represents a very substantial proportion of the time and cost involved in producing stereotype plates. Pages must be closed an appreciable length of time in advance of the time set for 30 operation of the press, and skilled workmen who might be otherwise engaged are required for the hand packing operation.

In the conventional process, the mat must be packed prior to the final forming and drying operation, and the 35 presence of the packing strips on the back of the mat during this operation creates further serious problems in the production of satisfactory stereotype plates. Particularly when the packed stereotype mats are subjected to the heat in the former and dryer, the packing shrinks 40 at a different rate and in a different amount than does the mat. In those areas where a large amount of packing has been applied, the unequal shrinkage and/or slippage between the mat and the packing due to the heat of the dryer may cause the strips to overlap printing areas or otherwise distort the mat. In addition, the packing strip with its adhesive layer does not permit free passage 45 of moisture and other vapors, and incomplete drying and irregular shrinkage of the mat often occurs in heavily packed areas. These deficiencies in hand packed mats 50 are particularly emphasized in color printing wherein registration of the several mats bearing the same imprint or reproduction is important. A slight variation in the manner of packing the several mats required for a single reproduction in color may seriously affect the registration 55 of material reproduced from such mats.

There is, therefore, a very great existing need for an 60 improved stereotype making procedure, and especially for an improved mat packing means which will not impede the free passage of moisture and other vapor through the back of the mat during drying and which will shrink substantially to the same degree as the mat. This material should also be flexible both before and after drying, since 65 the mat is subjected to considerable bending during use and must remain flexible during the treatment in the former and dryer, as well as at the time of the subsequent casting operation. Additionally, the combined mat and backing should also be capable of being bonded securely during the molding of the mat and held through the 70 process.

The mat backing should not restrict the forming of the mat. Unless the face of the mat is subjected to sufficient

pressure during the rolling and pressing of the mat, poor definition of the printing characters and a rough surface on the face of the printing will result. The desirable mat backing material should also be adaptable for use in conventional mat forming equipment and with conventional technique.

The present invention has for its principal object the provision of stereotype making procedures and materials capable of meeting the above stated requirements. A more specific object of the invention is the provision of an improved, composite stereotype mat and backing which can be used without any need for subsequent packing of the non-printing areas, while maintaining the normal vapor permeability necessary to the final forming of the mat. A further object is to provide such a composite mat wherein the shrinkage characteristics are compatible with existing stereotype mat products of the shrinkage type.

Another object of the invention is to provide a backing material suitable for use in conjunction with known stereotype mats, which is completely moldable and bondable with the mat to resist the molding pressures, and so that it can resist the pressures encountered during the forming and drying operation so as to be properly set to provide a unitary mat element having adequate strength and rigidity to withstand the pressures produced during the casting operation.

Still another object of the invention is to provide a method for the production of a finished stereotype matrix, which method is considerably faster in operation and more economical than the conventional process of hand packing stereotype mats now in use.

The various features of the invention and the specific manner in which the objects of the invention are accomplished will be made apparent in the following description and the accompanying drawings of certain illustrative embodiments of the invention.

In the drawings:

FIGURE 1 is a view in perspective of a portion of a lockup or other printing element illustrating one manner in which the mat, the backing, and the blanket are arranged in the practice of the invention;

FIGURE 2 is a view in perspective of a composite mat unit in accordance with the invention with the backing already attached;

FIGURE 3 is a fragmentary view in elevation of the assembly during pressing or molding of the mat about the printing form and is illustrative of one method which may be used;

FIGURE 4 is an enlarged cross-section view of a portion of the backed mat after its removal from the molding press;

FIGURE 5 is a fragmentary view of the backed mat during its formation in the dryer; and

FIGURE 6 is a side elevational view of the backed mat in the form in which it is received in a casting box.

In the practice of the present invention, a paperboard mat of the type now commonly used is provided with a backing consisting of a plurality of plies of creped, cellulosic tissues having dispersed therein a thermally rigidifiable binder, exemplified in the preferred embodiment of this invention by various thermosetting resins. A material of this type has been found to be properly moldable in that it is capable of taking a permanent set in the printing areas of the mat, but still retains its resiliency so as to provide the desired bulk in the portions overlying the nonprinting areas of the mat. Further advantages stem from the fact that the backing material, after hardening of the binder, has a substantially increased tensile and, of more importance, a substantially increased compressive strength, a desirable feature during the casting operation, but the mat is still quite flexible so that it can conform to the curved surface of the casting box. One of the more remarkable characteristics of the backing when applied to a conventional stereotype mat is the fact that the shrinkage of the combined mat and backing which

takes place during scorching is very nearly the same as the unpacked mat itself.

The material which we employ for the backing has found extensive use in the manufacture of filters and for various other purposes. The material and its method of preparation are described in Catlin and Wollwage U.S. Patent No. 2,554,814, issued May 29, 1951. As described in that patent, the preferred material consists of a plurality of plies of thin, creped, cellulosic tissue having an air-dry basis weight before creping within the range from about 5 to 10 pounds per standard ream of 480 sheets, each 24 by 36 inches, and having a crepe ratio generally in the range from 2.0 to 3.0, and containing a bonding agent in stated amounts.

The bonding agents which we prefer to use are liquid phenol formaldehydes. Other thermosetting resins such as urea-formaldehyde resins, melamine-formaldehyde resins, and resorcinol-formaldehyde resins, low pressure resins of the unsaturated polyester type (e.g. dialyl phthalate), and a mixture of such thermosetting resins may also be used.

It is important that the resins employed be curable at a fairly rapid rate. Most desirably, the resins should be curable at temperatures and times employed in conventional equipment for scorching stereotype mats. With the present invention the final drying and forming takes about three minutes and cures the resin at about 350° F. It will be apparent, however, that this temperature and time might be varied without any undue inconvenience or serious loss of time.

It is not essential that the resin impregnant be completely water soluble, as the resin can be introduced into the creped tissue sheets in solvents other than water or as a suspension of resin particles in water. In some instances, it is preferable to use a nonaqueous liquid vehicle, as there is less danger of reducing the bulk of the creped tissue than in the case of an aqueous vehicle. However, it is important that the impregnant be rendered sufficiently tacky by water to provide adequate adhesion between the several sheets and between the backing and the mat or flong. In this respect, it is believed that best results can be obtained with resins having a water tolerance or dilutability of from 1.0 part of water to 1.0 part of resin to 1.0 part of resin to 7.0 parts of water, by weight, in accordance with the standard dilutability tests used in the art.

The resin content in the impregnated product may vary depending upon the physical properties desired and the resin used. In general, for our purpose the product should contain from about 15 percent to 75 percent by weight of resin, with 40 to 50 percent being a particularly satisfactory range. The percentage values mentioned are on the weight of the finished product on a volatile-free basis. After impregnation and drying, the volatile content of the impregnated multi-ply material preferably should not exceed about 15 percent by weight, on a bone dry basis, as impregnated webs having higher volatile contents are hard to handle and become sticky. A volatile content of from 5 to 9 percent appears to provide the best results, although volatile contents of substantially lesser percentages may be satisfactory in certain instances where the flexibility of the impregnated web is not important and where an adhesive is to be used for joining the web to the stereotype mat. The volatile content of the material is determined by heating a sample for 10 minutes at 160° C., and measuring the weight loss. This loss, expressed as a percentage of the original weight, represents the volatile content.

Perhaps a more sensitive and more accurate test for determining a proper condition for the resin in the multi-ply backing material after impregnation and drying, if a water soluble resin is employed, is with reference to the water solubility of the resin. Expressed in this manner, it is preferable that the resin in the web after impregnation and drying be from 15 to 75 percent water soluble

in distilled water at 25° C. A water solubility of about 35% appears to provide the best results, but a considerable lower solubility, or even no water solubility, may be satisfactory if flexibility is not important and an adhesive is used for joining the web to the stereotype mat.

In a specific example, the backing was prepared by superposing twelve sheets of creped tissue made from chemical pulp, each individual sheet having a drier basis weight of 5.9 pounds per standard ream of 480 sheets, 24 by 36 inches, and a crepe ratio before impregnation of approximately 2.3. Thus the basis weight of the creped material was approximately 13.5 pounds per standard ream. The superposed sheets were impregnated by passage through a bath, aqueous or otherwise, containing the resinous bonding agent. The excess liquid was removed by passing the wet superposed sheets through felt covered squeeze rolls using only such pressure as would not change the structural characteristics of the multi-ply product or its individual plies. The impregnated sheets were then dried by a current of hot air at a temperature of about 245° F. to 325° F. The volatile content of the impregnated backing material at this stage was approximately 11 percent by weight. Material prepared in this manner can be readily heat treated to cure the resin dispersed throughout the plies of the material.

As normally practiced, the process of the present invention involves applying a relatively moist paperboard mat or flong of conventional type to the upper surface of a lockup containing the printing elements to be reproduced, while at the same time providing a multi-ply backing sheet of paper of the type described over the paperboard mat. This backing sheet may be integral with the mat or separate therefrom. Sufficient pressure is then applied to the assembly by conventional procedures, which may involve the use of a pressure pad or cushion, to produce a reproduction of the printing elements in the face of the mat. By this operation, the raised printing areas in the lockup become depressed areas in the face of the mat and the nonprinting areas in the lockup become raised areas in the mat.

After pressing, the mat and its associated backing are removed as a unit, and subjected to a drying operation in one or more steps. Drying of the mat serves to eliminate substantially all of the moisture in the mat so that the moisture does not interfere with the casting operation, while forming the mat for casting. Further, the drying and forming operation in connection with shrink-type mats serves to reduce the size of the mat to the particular dimensions required in the stereotype plate. During the drying process, the temperature is maintained at a sufficiently high value to set the resin in the backing to effect polymerization to such a degree that the resin no longer exhibits any substantial plastic flow under the temperatures and pressures of plate casting.

In FIGURE 1, reference numeral 10 indicates generally a printing form including the usual heavy metal chase 11 for containing the various components of the form, including the usual locking wedges of quoins (not shown) for holding the printing elements in place in the case. Substantially flush with the level of the chase 11 is an arrangement of printing elements which may include type slugs 12, each of which contains raised type faces 13 and engraving 14 separated from the type 12 by means of a spacer 16 and a second set of type 17 with its raised type faces 18. A paperboard mat 19, which ordinarily contains from about 10 to 40 percent by weight of free moisture is shown superposed over the printing form. Paperboard mats of this type commonly vary in thickness from about .024 to .040 inch. The mats are selected by a given newspaper primarily on the basis of their shrinkage characteristics. Mats of the type now most generally used shrink considerably upon drying, depending in part upon their relative moisture content. This shrinkage occurs to the greatest degree transversely of

the mat, at right angles to the machine direction of the fibers. The shrinkage in the lengthwise direction is ordinarily about half of what it is in the cross direction.

In newspaper work, it is common to use mats which provide from about one-half to about one and one-fourth inches in cross-wise shrinkage for a mat measuring about fifteen and nine-sixteenths inches wide and twenty-one and three-quarter inches long between the limits of the type area. In choosing a mat for the process of this invention where only one drying step is used, it may be desirable to allow for a slight decrease in shrinkage over that ordinarily anticipated, so that where a given mat may have a characteristic shrinkage of one and one-eighth inches, it will shrink about one inch when combined with the backing material described. Where a conventional pre-drying step is employed, however, substantially all of the rated shrinkage in a given mat will be achieved by the end of the final drying step.

Disposed immediately over the mat 19, and coextensive therewith is a pad or multi-ply sheet 21 composed of a plurality of bonded plies of creped cellulosic tissue or wadding impregnated with an unset thermosetting resin, as previously described. For a mat having a thickness of .024 to .040 inch and a moisture content of 10 to 40 percent, the initial thickness of the wadding pad should be in the range of from about .030 to .100 inch. This is equivalent to a sheet of from 6 to 20 plies of resin impregnated tissue, as described, having a basis weight per standard ream of about 100 to 300 pounds and containing 40 percent of resin on a bone dry basis. It may be desirable to use a non-impregnated tissue ply above the resin impregnated plies to avoid adherence between the backing and the molding combination.

Above the wadding pad 21 is a compressible cushion or molding combination 22 which may comprise a sheet of yieldable material such as cork, or mixtures of cork and synthetic rubber and/or fabric. In this respect it should be noted that the molding combination fairly well regulates the pressure that is applied to the stereotype mat during the molding operation. The pressure on the mat will vary considerably between the printing and nonprinting areas because of the type of molding combination selected and because of the space areas and depths available in the lockup. Consequently, it will be seen that the molding combination is a matter of choice depending largely on the space-depth desired in the mat and on the particular type of mat being used.

One example, of the numerous molding combinations which could be employed includes a sheet .070 inch thick consisting of a cork composition with a fabric facing, in combination with a fiberboard sheet having a thickness of .090 inch. However, we have found that the molding combination can be eliminated in some cases.

In the practice of the invention by the use of the materials described in the foregoing, it will generally be found that good adhesion is produced between the mat and the plies of the backing material. This is especially true when the backing material contains a moisture sensitive resin and when the volatile content of the mat material is greater than about 4.0 percent.

In certain instances, however, it has been found desirable to provide an additional layer of adhesive between the mat and the backing. This adhesive may be of such nature that it adheres the mat and the backing prior to the molding operation, or the adhesive may be applied in such manner that it joins the mat and the backing only during the molding and/or drying operations. For example, an adhesive may be applied to the mat or to the backing, or to both, or the adhesive may consist of a separate film or an impregnated carrier sheet adapted for insertion into the lay-up assembly between the mat and the backing.

The adhesive coating 20a is preferably a uniform film of a moisture sensitive adhesive material, such as sodium acrylate, "Methocel," a methyl cellulose sold by Dow Chemical Co. or polyvinyl alcohol, in order that it will

be tacky during the formation of the combined mat and backing when the moisture in the mat is drawn into the backing, or it may be a pressure sensitive material which will bond the backing to the mat during the molding operation. Further, the adhesive should be moisture permeable, so that it does not act as a barrier to the moisture in the mat 19a as this moisture seeks to penetrate the backing 21a.

The adhesive selected for joining the mat to the backing should preferably be one which is sufficiently tacky to provide a good bond between the mat and the backing during the molding of the composite stereotype mat. Otherwise, the subsequent drying operation might deform the backing as it receives moisture from the mat and cause uneven shrinkage of the two resulting in their getting out of register with each other.

If desired, a film or carrier sheet may be used for the adhesive film 20a. However, in such instance it is desirable that the carrier sheet be capable of distortion in order to conform with the mat and backing. For this reason a soft tissue or a non-woven fabric might be used.

It is possible that by using an added adhesive layer, as described above, a somewhat smaller amount of resin might be used in the backing, since this resin content is no longer relied on for adhering the backing to the mat in the manner previously described. It is also possible that it may be desirable in certain instances to use a heated pressure roll in the molding operation, in order to better set the adhesive and thereby improve the bonding between the mat and backing.

With reference now particularly to FIGURE 3, it is seen that the printing form 10 with the mat, backing, and blanket in place is set on the table 23 and passed between the nip of pressure rolls 24 and 26. One or both of the rolls 24 and 26 is made vertically adjustable to compensate for different thicknesses of printing forms. The pressures of molding used in our process are substantially the same as those used presently in molding stereotype mats. It is difficult to measure the exact pressure employed, as the contacting areas of roll to which the pressure is applied cannot be ascertained accurately. However, it is generally accepted that the molding pressures required for good reproduction are on the order of 2,000 to 4,000 pounds per square inch over the printing areas and may be considerably higher.

The use of a roller molding machine comprising a chase-supporting bed and a pair of rotatable pressure rolls is by far the most common method of molding mats, but the process of the present invention is equally applicable to molding procedures involving the use of direct pressure with flat platens.

As pressure is applied to the assembly shown in FIGURE 3, the mat 19 is compressed into the spaces between the raised printing characters and forms a sharply defined reproduction of the printing characters contained in the lockup or form 10. The porous backing 21 is also capable of absorbing any moisture expressed from the mat 19. The backing 21 is considerably more compressible than the mat 19 and, as a result of the pressing, the thickness of the backing 21 is considerably reduced over the printing areas. Under ordinary molding pressures, the thickness may be reduced by a factor of four or five times over the printing areas, so that a backing originally .050 inch in thickness may end up as a compressed backing of about .010 inch, whereas in the nonprinting areas the bulk is compressed to about .040 inch, thereby providing a space depth between the level of the nonprinting areas and the base of the printing areas of about .030 inch. Thus in one operation the mat is molded and completely packed simultaneously and more rapidly than is possible in a hand packing operation. Furthermore, with the described invention, the molded depth retention in half tone areas is better than in a hand packed mat.

The backing material is such that its face is able to

conform accurately to the contour of the back of the mat 19 during application of pressure. At the same time the backing becomes quite securely bonded to the back of the mat 19 over the areas of the mat subjected to high molding pressures. In instances where the glue line or adhesive coating 20a is not relied on to bond the backing to the mat, this bonding is effected either because of the adhesive properties of the resin contained in the backing, or it may be partly due to a mechanical locking of the printing areas at the back of the mat in the collapsed areas of the backing immediately overlying these areas of the mat. With the use of the adhesive coating 20a the pressure on the mat during the molding operation causes the back to be bonded to the mat. With a moisture sensitive adhesive this bonding is effected by the expression of moisture in the mat toward the adhesive to thereby render the latter sufficiently tacky to bond the backing to the mat.

A portion of the backed mat after removal from the molding apparatus is illustrated in enlarged form in FIGURE 4. As seen in that drawing, the face of the mat 19 is depressed in conformity to the shape of the lockup, as seen at 28 and 29, depending on the pressure, molding combination, and the space areas and depths available in the original lockup.

In the nonprinting areas, as for example in the area 29, the remarkable resiliency of the backing 21 causes the backing to recover much of its original thickness after removal of the molding pressure, as indicated at numeral 33. Yet in the areas above the printing surfaces, such as the area 31, the backing takes a more permanent set but still retains a high degree of flexibility and moisture permeability. The result is that the backed mat produced by the molding operation has a generally planar rear surface 35 which may be readily conformed to the surface of the dryer. Further, the backing material is packed into those small nonprinting areas that a hand packer does not even touch in the ordinary process of stereotype mat forming. Consequently, there is provided by the backing a proper arrangement of bulk for resisting collapsing of the mat during subsequent steps in the formation of the finished stereotype matrix.

After the removal from the molding apparatus, the composite mat and backing is then ready for drying and for setting of the resin. For the manufacture of curved stereotype plates, the mat 19 and its backing 21 are given a uniform curvature by introducing the mat into a conventional dryer assembly illustrated in FIGURE 5. The particular dryer illustrated in the drawings consists of an asbestos covered drum 34 in which a plurality of heating elements 36 are disposed beneath the asbestos surface. A cover or chamber 37 having a perforated inner face 38 is hinged to the base 34 at a hinge 39. The backed mat is held against the inner face 38 by applying a vacuum to the back of the composite mat through the perforations in the face 38. The cover is also heated by means of spaced heating elements 40 contained therein. As previously stated, the multi-ply pad of resin-impregnated tissue sheets may include one unimpregnated ply on the upper surface thereof.

The vacuum applied to the mat holds the mat in contact with the face 38 and spaces the face of the mat slightly from the asbestos covered surface of the base 34 when the cover 37 is in its closed position. Thus the vacuum serves not only to hold the mat in position but, also, forms the back of the mat in a smooth surface so as to provide a uniformly curved reference surface for the mat. The temperature at the base of the scorcher is ordinarily on the order of 250° to 400° F. As the heat is applied, the moisture is driven from the mat and this moisture passes through the porous backing material and is thereupon vented. It is important that the resin selected should not become cured or rigid until substantially all of the desired shrinkage of the mat and backing has taken place. Consequently, the resin should be one which will become

cured throughout at a temperature somewhere near the upper range of the scorch temperature which will prevail throughout the mat when essentially all of the moisture has been drawn therefrom. The resins mentioned above have these characteristics and mats packed with these types of dispersed resin products do not evidence any tendency to crack or warp during casting of the stereotype plate.

Where only one drying step is used, a treatment time of 2 to 5 minutes at temperatures of 300° F. to 400° F. will suffice to drive off the moisture and set the resin sufficiently under moisture conditions normally prevailing in that mat. The control of shrinkage is facilitated by operating at a lower vacuum, on the order of one and one-half inches of mercury during the first minute or two and then increasing it to a value of 5 to 6 inches of mercury when substantially all of the moisture has been driven off. And, as previously mentioned, substantially all of the moisture is driven off before the resin in the backing is set and, therefore, such resin content does not interfere with the shrinkage of the mat and backing as a unit. Where a pre-drying step is employed in conjunction with a final drying and forming, times of about 40 to 80 seconds at temperatures of about 150° to 250° F. may be employed to initiate shrinkage of the composite mat without substantial setting of the resin. In this latter respect, it should be noted that there are definite advantages in some instances in utilizing a pre-drying step before finally forming the mat. The pre-drying operation helps to rigidify the backing so that it is better able to resist the vacuum pressure in the final dryer and prevent an undesirable collapsing of the uncured mat under such pressure. Further, this pre-drying of the mat and backing is an aid in providing better space-depth characteristics in some instances.

The resin in the backing should be cured sufficiently during the final drying operation to a point wherein it will resist collapse under the temperatures and pressures encountered in the casting of the stereotype plate. Our experience indicates that in the case of a phenol-formaldehyde resin a cure of at least 85 percent should be achieved. Expressed alternatively, the resin extractibles in the sheet should not exceed about 15 percent. The extractables content can be readily determined by the standard A.S.T.M. test (D494-41) which involves taking a known weight of typical sample of the cured sheet material in finely comminuted form, and placing this sample in a Soxhlet apparatus where it is extracted with hot acetone for a period of four hours. The acetone is then evaporated under controlled conditions and the sample removed, so that the residue constitutes the extractable materials which have been dissolved by the acetone.

Upon removal of the backed mat from the scorcher, the mat is ready for insertion in the casting box. The final form of the mat is illustrated in FIGURE 6 of the drawings and includes the paperboard mat 19 having a casting face 19b of concave shape and the backing 21 in which the thermosetting resin has become set and rigidified by the heat treatment in the dryer. Composite mats of this type have been found to adequately resist collapse under type casting pressures on the order of 15 to 25 pounds per square inch.

The process described can be very conveniently carried out on conventional stereotype forming equipment with little or no change in the present procedures or equipment and, when so used, it realizes most important savings in time and labor as well as producing an improved mat and, consequently, a better printing plate.

There are a number of factors which should be considered in the practice of the invention in order to achieve the best results in the molding of the composite mat and backing. These include (1) the degree of creping in the individual unimpregnated tissue plies constituting the backing material; a crepe ratio of between 1.3 and 2.5 is preferred, (2) the amount of stretch in the backing after

impregnating and drying should be between 20% and 60% in the machine direction, based on the original length of the sample of backing, (3) the resin content in the backing, which is preferably 40 to 50 percent by dry weight of the finished product on a volatile free basis, but which may be within a range of 15 to 75 percent and still be effective in certain instances, (4) the thickness or bulk of the backing, preferably .030 to .100 inch before the composite mat is formed in the case of newspaper mats, (5) the water solubility of the resin in the backing after impregnation and drying which is desirably about 35%, in the event a water soluble resin is used, (6), the percentage of volatiles in the backing after the composite web is formed, indicated above as being preferably no greater than 15 percent of the resin content, with a range of from 5 to 9 percent being desired for most practical uses, (7) the type of molding combination employed, and (8) whether a single or multiple step, non-shrink or shrinkage process is desired in forming the stereotype mat or matrix. It will be understood of course, that the thickness of the mat will be largely a matter of convenience. While all of the above mentioned factors play a part in providing the improved stereotype mat made possible by this process, a proper balancing within the various ranges disclosed herein should be achieved to obtain the finest quality reproduction.

The foregoing discussion has dealt primarily with the backing of curved stereotype mats of the high shrink type now commonly employed in newspaper work. The numerous advantages of the new combination can also be realized in related fields. As previously indicated, the mat and backing can be pressed between flat platens, and the resulting backed mat after curing of the resin and shrinkage of the mat can be employed for making flat castings. Alternatively, the molding, curing, and shrinkage may be part of the same operation, by employing heated, perforated platens in the flat molding press.

For another example, advertising agencies distribute the so-called "ad mats" to numerous newspapers throughout the country. These mats are commonly of the "no-shrink" type and are intended to provide a mold for receiving a flat casting of metal or for direct casting in newspaper work. The casting is then inserted into a newspaper page lockup along with the remaining printing elements, and a high shrinkage mat is then molded on this lockup. The described backing can also be employed as a backing for the no-shrink type mat. In this type of application, the resin in the backing is conveniently cured at the time the mat is molded by using heated platens in a direct pressure molding assembly, and the mat and its attached backing may then be distributed to the various newspapers.

Another field in which mats of little or no shrinkage are commonly employed is that of color reproduction. Normally, color printing systems include a series of as many as four printing rolls, one for each of colors desired, so that a plurality of stereotype plates must be provided for each printed page. In this field, it is essential that there be perfect registry between the printing surfaces, so it is common practice to use a no-shrink mat for preparing each of the plates. Because of its inherent ability to conform exactly to the mat during drying the backing material of the present invention has especial utility in the manufacture of such mats.

It will be evident that various modifications can be made in the disclosed examples without departing from the scope of the present invention.

We claim:

1. The method of making a stereotype mat which comprises applying onto a printing form a relatively moist paperboard mat having a moisture content in the range from 10 to 40 percent by weight and a multi-ply backing superimposed thereon, said backing comprising a moldable sheet containing a plurality of plies of creped tissue having an unset thermosetting resin dispersed therein, the

resin content in said backing sheet constituting from 15 to 75 percent by weight of said sheet on a dry basis, said backing sheet having a volatile content in the range from 5 to 15 percent by weight on a bone dry basis, applying sufficient pressure to the resulting assembly to form an impression of the printing areas of said printing form into said mat, removing said assembly from said printing form, drying said backing and said mat while applying a reduced pressure at the rear of said backing so that the moisture in said mat is vented through said backing, and heating said mat and said backing under conditions sufficient to cure the resin in said backing to withstand the pressures encountered in stereotype casting.

2. The method of making a stereotype mat which comprises applying onto a printing form a relatively moist paperboard mat having a moisture content in the range from 10 to 40 percent by weight and a multi-ply backing superimposed thereon, said backing comprising a moldable sheet containing a plurality of plies of creped tissue having an unset thermosetting resin dispersed therein, the resin content in said backing sheet constituting from 15 to 75 percent by weight of said sheet on a dry basis, said backing sheet having a volatile content in the range from 5 to 15 percent by weight on a bone dry basis, applying sufficient pressure to the resulting assembly to form an impression of the printing areas of said printing form into said mat, removing said assembly from said printing form, drying said backing and said mat so that the moisture in said mat is expelled, and heating said mat and said backing under conditions sufficient to cure the resin in said backing to withstand the pressures encountered in stereotype casting.

3. The method of making a stereotype mat which comprises applying onto a printing form a relatively moist paperboard mat having a moisture content in the range from 10 to 40 percent by weight and multi-ply backing superimposed thereon, said backing comprising a moldable, moisture-permeable sheet containing a plurality of plies of creped, cellulosic tissue having an unset thermosetting resin dispersed therein, said backing sheet containing from 15 to 75 percent by weight of said resin on a dry basis, said backing sheet having a volatile content in the range from 5 to 15 percent by weight on a bone dry basis, applying sufficient pressure to the resulting assembly to form an impression of the printing areas of said printing form onto said mat, removing said assembly from said printing form, drying said mat and said backing under conditions sufficient to permit shrinkage of said mat and backing to a predetermined degree, and heating said mat and said backing at temperatures sufficient to cure the resin in said backing.

4. The method of making a stereotype mat which comprises applying onto a printing form a paperboard mat having a free moisture content in the range from 15 to 40 percent by weight and a multi-ply backing sheet or pad superimposed thereon, said backing comprising a plurality of plies of creped paper bonded together by an unset thermosetting composition distributed through said plies and having an initial thickness in the range of from about 0.030 to 0.100 inch and being moisture permeable, the resin content in said backing material constituting from 15 to 75 percent by weight of said backing material, said backing sheet having a volatile content in the range from 5 to 15 percent by weight on a bone dry basis, applying sufficient pressure to said mat and said backing while in superimposed relation over said form to form an impression of said form in said mat, removing said mat and backing material as an assembly from said printing form, and thereafter drying said mat and said backing at a temperature sufficient to dry said mat into a substantially moisture-free condition and to cure the resinous composition in said backing material.

5. The method of making a stereotype mat which comprises impregnating a plurality of plies of creped, cellulosic tissue with an unset thermosetting resinous compo-

sition dispersed in a liquid vehicle, drying the impregnated material to provide a laminated, moisture-permeable backing material having resin particles dispersed therein in sufficient quantities to provide a resin content of from 15 to 75 percent by weight in said backing material, said backing material having a volatile content in the range from 5 to 15 percent by weight on a bone dry basis, superimposing said backing over a paperboard mat with an adhesive film therebetween, said paperboard mat having a moisture content from 10 to 40 percent by weight, laying the resulting backed mat over a series of printing elements with the paperboard portion thereon in contact with said element, applying sufficient pressure to make an impression of said printing elements in said paperboard, removing said backed mat from said printing elements, and thereafter drying said backed mat by the application thereto of heat, while simultaneously removing moisture vapor from said mat through said backing material, at a temperature sufficient to dry the backed mat and to cure the resin in said backing material sufficiently to withstand the pressures encountered in stereotype casting.

6. A stereotype matrix comprising a molded flong and a molding blanket secured thereto and providing a backing for said flong, said molding blanket including a cured thermosetting resin impregnated fibrous sheet, the free surface of said flong having the printing matter molded therein and the contacting surfaces of said blanket and said flong being contoured in the non-printing areas, the free surface of said molding blanket being flat.

7. A stereotype matrix comprising a molded flong and a molding blanket in juxtaposition, and a quantity of adhesive between said flong and said molding blanket adhering said molding blanket to said flong, said molding blanket including a sheet of fibrous material impregnated with a cured phenolic resin, the free surface of said flong having printed matter molded therein and the contacting surfaces of said sheet and said flong being contoured in the non-printing areas, and the free surface of said molding blanket being flat.

8. A stereotype matrix comprising a molded flong and a molding blanket in juxtaposition, and a layer of adhesive between said flong and said molding blanket adheiring said molding blanket to said flong, said molding blanket consisting substantially of a layer of paper sheet material impregnated with a cured phenolic resin, the free surface of said flong having printed matter molded therein and the contacting surfaces of said blanket and said flong being contoured in the non-printing areas, the free surface of said molding blanket being flat.

9. A stereotype matrix comprising a molded flong and a molding blanket in juxtaposition, and a layer of adhesive between said flong and said molding blanket adheiring said molding blanket to said flong, said molding blanket consisting substantially of a layer of paper sheet material impregnated with a cured phenol formaldehyde resin, the free surface of said flong having printed matter molded therein and the contacting surfaces of said blanket and said flong being contoured in the non-printing areas, the free surface of said molding blanket being flat.

10. A stereotype matrix comprising a molded flong and a molding blanket in juxtaposition, and a layer of adhesive between said flong and said printing blanket adheiring said molding blanket to said flong, said molding blanket consisting substantially of a layer of paper sheet material, having a maximum thickness of between about 0.035 inch and about 0.040 inch and impregnated with a cured phenol formaldehyde resin, the resin constituting about 50% by weight of the impregnated sheet, the free surface of said flong having printed matter molded therein and the contacting surfaces of said blanket and said flong being contoured in the non-printing areas, the free surface of said molding blanket being flat.

References Cited in the file of this patent

| UNITED STATES PATENTS |                  |               |              |
|-----------------------|------------------|---------------|--------------|
| 815,999               | Annand           | May 27, 1909  | 2,111,205    |
| 1,233,298             | Baekeland        | July 17, 1917 | 2,343,930    |
| 1,398,142             | Novotny          | Nov. 22, 1921 | 5 2,492,348  |
| 1,524,155             | Schroger         | Jan. 27, 1925 | 2,554,814    |
| 1,726,151             | Hole             | Aug. 27, 1929 | 5 2,587,833  |
| 1,960,697             | Cochran et al.   | May 29, 1934  | 2,703,051    |
| 2,041,941             | Matuschke et al. | May 26, 1936  | 10 2,771,646 |
| 2,070,293             | Morgan et al.    | Feb. 9, 1937  | 461,045      |

|               |       |               |
|---------------|-------|---------------|
| Catlin        | ----- | Mar. 15, 1938 |
| Rowe          | ----- | Mar. 14, 1944 |
| Baker         | ----- | Dec. 27, 1949 |
| Catlin et al. | ----- | May 29, 1951  |
| Germain       | ----- | Mar. 4, 1952  |
| Richardson    | ----- | Mar. 1, 1955  |
| Schaum        | ----- | Nov. 27, 1956 |

## FOREIGN PATENTS

|         |       |               |
|---------|-------|---------------|
| Germany | ----- | June 11, 1928 |
|---------|-------|---------------|